

Patented Dec. 15, 1925.

1,565,994

# UNITED STATES PATENT OFFICE.

GEORGE K. FRANKLIN, OF SWEDESBORO, NEW JERSEY.

NONCORROSION COMPOSITION FOR TERMINAL BATTERIES.

No Drawing.

Application filed April 7, 1925. Serial No. 21,318.

To all whom it may concern:

Be it known that I, GEORGE K. FRANKLIN, a citizen of the United States, residing at Swedesboro, in the county of Gloucester and State of New Jersey, have invented new and useful Improvements in a Noncorrosive Composition for Terminal Batteries, of which the following is a specification.

My invention relates to a new and useful improvement in a non-corrosive composition for battery terminals and the process of producing the same, and has for its object the provision of a composition or material in the form of a paste to be applied to the terminals of automobile or other similar batteries which will stop or reduce to a minimum the chemical action which often takes place about battery terminals so as to prevent said terminals from corroding.

A further object of the invention is the production of a non-corrosive composition by a process which consists of making a mixture of baking soda and graphite and make a second mixture of ammonia, carbolic acid, lubricating oil and alcohol and then adding one mixture to the other and stirring or working the conglomerate into a thin smooth paste.

In producing the composition I first mix together five parts of baking soda, two and one-half parts of graphite and also separately mix two parts of ammonia, one part of carbolic acid, one part of lubricating oil and one part of alcohol, these two mixtures are then combined or one added to the other and the resulting conglomerate thoroughly mixed together by stirring, agitating or

working until a thin smooth paste is produced.

The composition set forth above produced by the process described is used by applying a small amount of paste to the terminals of an automobile or other batteries and the application thereof will stop or reduce to a minimum any chemical action which might take place about said terminals and therefore prevent the same from corroding thus keeping the terminals always in good condition and prolonging the life thereof.

Having thus fully described my invention, what I claim as new and useful is:—

1. A composition resulting from the combination of two mixtures, one of said mixtures including baking soda and graphite and the other mixture including ammonia, carbonic acid, lubricating oil and alcohol.

2. A non-corrosive composition resulting from the combining of a mixture consisting of five parts of baking soda, and two and one-half parts of graphite with another mixture consisting of two parts of ammonia, one part of carbolic acid, one part of lubricating oil and one part of alcohol.

3. The process which consists of mixing baking soda and graphite, then separately mixing ammonia, carbonic acid, lubricating oil and alcohol, then combining or mixing the resultants of the first two mixtures and then working the conglomerate into a thin smooth paste.

In testimony whereof, I have hereunto affixed my signature.

GEORGE K. FRANKLIN.